# EUROPEAN PATENT SPECIFICATION

(11) **EP 0 065 749 B1**
(45) Date of publication and mention of the grant of the patent: **19.12.1984**
(21) Application number: 82104370.0
(22) Date of filing: 18.05.1982
(51) Int. Cl.: D21B 1/06

(54) **Method for manufacturing a starting material suitable for further processing to absorbent products**
Verfahren zur Herstellung eines Anfangsmaterials geeignet zur Weiterverarbeitung zu absorbierenden Produkten
Procédé pour la fabrication d'une matière de départ propre à être transformé en des produits absorbants

(30) Priority: 20.05.1981 SE 8103172
(43) Date of publication of application: 01.12.1982
(73) Proprietor: Mo och Domsjö Aktiebolag, S-89101 Örnsköldsvik (SE)
(72) Inventor: Lindahl, Jonas Arne, S-89200 Domsjö (SE)
(74) Representative: Barz, Peter, Dr.

## Description

The present invention relates to a method for the conversion of web-dried pulps intended for the manufacture of absorbent products. By pulp is meant here and in the following cellulose pulps, such as chemical, chemi-mechanical and mechanical pulps. Examples of such cellulose pulps include sulphite and sulphate pulps, refiner mechanical pulp, and groundwood pulps. The invention can thus be applied to practically all kinds of web-dried pulps.

In the manufacture of absorbent products, pulp fibres produced from different lignocellulosic materials are used in large quantities. The fibres are packed solidly together in sheet form, in bales or reels. The sheets packed in bales normally have a length from 400 to 800 mm, a width of from 300 to 800 mm, a grammage of from 600 to 900 g/m², and a density of from 700 to 900 kg/m³ (bale pulp). In principle, reels comprise extremely long pulp sheets cut into widths which normally vary from 100 mm to 150 mm (reel pulp), with a density of from 600 to 750 kg/m³. It is also known in the manufacture of absorbent products to use as the starting material therefor a pulp which, prior to being dried, is wet shredded into flakes (flake pulp). Prior to being dried, the flakes have a dry solids content of about 50%. After drying the flakes to a dry solids content of from 85 to 92%, they are pressed into decimeter-thick slabs, which because the hemicellulose acts as an adhesive are extremely hard and difficult to break up. The slabs have a density in the order of 550-800 kg/m³. The flake pulp also contains a large amount of nodules. Flash-dried slabs are delivered in the form of bales having a height which varies from 300 mm to 1200 mm.

In the manufacture of absorbent products, the reel pulp or bale pulp is shredded and disintegrated into a voluminous fluff. One problem with the dry shredding of bale pulp is that it is difficult to achieve uniform production. Moreover, it is difficult to obtain a uniform dry solids content, owing to the fact that the bales are made up of relatively large separate units, in the form of sheets or slabs. In the handling of normal bales, powerful shredders are required which, in order to function satisfactorily, demand a given minimum production. Consequently, manufacturers of relatively small quantities of absorbent products can scarcely use bale pulp, but are referred to the more expensive reel pulp. In addition to the requirement of a minimum production for optimal use of the aforesaid shredders, the investment costs involved are unrealistically high in the case of those manufacturers using relatively small quantities of bale pulp.

The shredders used to shred reel pulp are simpler than those used to shred bale pulp. Reel pulp functions relatively satisfactorily from the aspect of process techniques. One disadvantage with reel pulp, however, is that it is costly to produce in the pulp mills, because it requires a longer drying time in order not to be too hard. Reel pulp demands a market price which is about $100 per ton above that of bale pulp.

The aforementioned problems are solved by means of the present invention. Accordingly, the invention relates to a method for manufacturing a cellulose pulp material suitable for further processing to absorbent products, in which method dried cellulose pulp web is used as basic material. The method is characterized by disintegrating the dried cellulose pulp web to flake form directly in the pulp mill, and by compressing the resultant flakes into large easily handled and transportable units having an apparent density of 200-800 kg/m³, preferably 300-700 kg/m³.

Thus, the obtained flakes are compressed into larger units already in the pulp mill in order to bring them to a form in which they can be readily handled and readily transported to a converting plant.

It has also been found especially suitable for the dried pulp web to have a dry solids content of at least 80% prior to being disintegrated, disintegration suitably being effected by tearing, so that subsequent to being torn at least 70% of the pulp is in the form of pieces whose diameter, or length, and width vary between 2 mm and 70 mm, preferably between 3 mm and 40 mm. The remaining parts of the pulp have sizes lying outside these ranges. Prior to the manufacture of the aforementioned absorbent products, the thus produced flake-containing units are shredded in a converting plant in a manner known per se, using known apparatuses. Because of the good disintegrating properties exhibited by the starting material produced in accordance with the invention, shredding can be effected much more readily than with known bale pulps.

When carrying out the method according to the invention it has been found an advantage to cut the dried cellulose pulp web into sheets prior to disintegrating the pulp into flakes, and to stack the sheets loosely on top of each other, whereafter the sheets are cut into strips which, in turn, are disintegrated into flakes, which are then compressed to form larger units. Alternatively, the dried cellulose pulp web can be disintegrated directly upon leaving the drying machine to flake form, i.e. without being cut into sheets, the flakes then being compressed to form larger units. This latter alternative is to advantage insofar as it obviates the need for sheet-manufacturing apparatus and apparatuses for stacking and cutting the sheets.

Considerable savings in energy are afforded by the invention compared with the energy consumed when converting bale pulp to fluff using conventional methods. Furthermore, when practising the method according to the invention it is possible to eliminate the customary manufacture of sheets and the pressing of said sheets in the pulp mill, and instead to directly convert the dried pulp web into flakes by means of a simple spiked roller and to then compress the flakes into larger, readily transportable units of desired density. The greater bulk of the starting material produced according to the invention also results in a reduction in the consumption of wood raw materials. The invention also enables small manufacturers of absorbent products to transfer to the use of less expensive pulp as a starting material, and also obviates the need for certain equipment, such as powerful guillotines and shredders.

The invention is illustrated in the following Examples which represent preferred embodiments and each of which is compared with tests carried out in accordance with conventional techniques.

### Example 1

In a sulphite mill, in which there was produced a 2-stage-cooked fully bleached spruce sulphite pulp having an intrinsic viscosity of 1100 cm³/g and a brightness of 93% ISO, there was installed downstream of a drying machine an apparatus, a so-called guillotine, for cutting bales of pulp sheets into strips. The sheets were loosely stacked one upon the other without being compressed, whereafter the sheets were cut into strips by means of the guillotine. The strips had a width of 5 cm and a length of 80 cm. The dry solids content of the pulp immediately after the web dryer was 93%. The pulp strips were carried on a belt conveyor to a hammer mill, in which the strips were reduced to flakes having an average length of about 20 mm and an average width of about 15 mm. The pulp flakes were passed to a slab press and then to a bale press. In this test large units in the form of bales having a weight of 180 kg bone dry pulp were produced. The bales had straight sides, and a height of 47 cm, a length of 91 cm and a width of 65 cm. This resulted in a bale density of 650 kg/m³ for each bale. After being conditioned for two weeks, the flake bales were transported to a converting plant for the manufacture of diapers. The bales had a dry solids content of 91.5%. The bales of flakes were opened in the converting plant and shredded into small pieces by means of a simple peg shredder. These pieces were identical in size and number to the flakes obtained prior to baling in the pulp mill. The pulp flakes were conveyed in a screw conveyor to a disc refiner where they were defibrated into fluff. It was noted during this test that the flake bales could be torn apart with ease and the pulp flakes readily defibrated. It was also noted that problems caused by static electricity were considerably less than normal. During the test, diapers having a weight of about 32 g were manufactured. The diaper weight-spread amounted to ±1 g, and was fully satisfactory. The bulk of the pulp and its absorption properties were checked prior to manufacturing the diapers. The results are given in Table 1 below.

In order to make a comparison there were taken from the mill pulp sheets which had been stacked and compressed to bale form in a conventional manner and which had the same measurements as those mentioned above. The bales had a weight of 190 kg (bone dry) and a density of 685 kg/m³. The dry solids content of the pulp immediately after the web dryer was 93%. After being conditioned for two weeks, the dry solids content was 92.0%. The pulp bales were then transported to the converting plant, where they were cut into strips on a guillotine. The strips had a width of 5 cm and a length of 80 cm. The pulp strips were conveyed on a belt conveyor to a hammer mill, where they were reduced to flakes having an average length of about 20 mm and an average width of about 15 mm. The pulp flakes were conveyed with screw conveyors to a disc refiner, where they were defibrated. No difficulties were experienced in manufacturing diapers from the defibrated fluff pulp, with the exception of certain problems arising from static electricity. During the test, diapers having a weight of about 32 g were manufactured. The diaper weight-spread was ±1 g.

The bulk of the pulp and its absorption properties were checked directly after the defibrating stage, i.e. just prior to the diaper manufacturing stage. The results are given in the Table below. All measurements have been made according to SCAN-C 33:80.

As will be seen from the Table, the amount of energy consumed when practising the method according to the invention was surprisingly less than that consumed when practising the conventional method. Although no positive explanation can be given as to why this surprising result was obtained, one possible theory is that in the case of flake-containing bale units produced in accordance with the invention the fibre-to-fibre bonds between the flakes developed during said storage period are weaker and also smaller in number. It will also be seen from the Table that the pulp manufactured in accordance with the invention has a higher bulk, which makes it possible to manufacture products of unchanged volume but with the use of lesser weight-quantity pulp, i.e. it is possible to save pulp and therewith wood starting materials. Another surprising and positive effect is that the absorption capacity of tho pulp i( not impaired as _{]} result of the lower number ot fibres per unit of volume. The good absorption rate has also been maintained.

### Example 2

In the same mill as that referred to in Example 1 the sulphite pulp was mixed with 25% flash dried spruce groundwood pulp having a freeness CSF of 300 ml and being bleached with hydrogen peroxide to a brightness of 73% ISO. The groundwood pulp was converted in a pulper to a suspension with a pulp consistency of 3%, which was diluted and charged to the head box of the wet machine simultaneously with the sulphite pulp, whereafter the mixed pulp was dried in the drying section of the wet machine to a dry solids content of 93%. The resultant pulp sheets were loosely stacked one upon the other without being compressed, and cut into strips on a guillotine, torn into flakes in a hammer mill and pressed into large units in the form of bales having straight sides in the same manner as in Example 1.

When admixing 25% groundwood pulp, the weight of the bales dropped to 150 kg bone dry pulp and the mean density of the bales to 528 kg/m³. The bales were stored for conditioning for two weeks, to equalize the moisture contents. The bales were then transported to the converting plant, where diapers were manufactured in the same manner as that described in Example 1. Samples were taken for measuring brightness, bulk, absorption properties and the average weight of the diapers. The results are set forth in Table 2 below, which also shows the total energy consumed in the tearing and defibrating operations.

For comparison purposes, a test was carried out using conventional techniques. In the comparison tests there was used a sulphite pulp similar to that previously used, which was mixed with 25% of the peroxide-bleached spruce groundwood pulp, which had been flash dried to a dry solids content of 90% and had the form of bales each containing five slabs, each slab having a height of 9 cm. In mixing one slab of groundwood pulp was stacked on each bale of sulphite pulp. The mixed bale was then cut into strips of 5x80 cm in size on the guillotine and conveyed on a belt conveyor to a hammer mill, where the strips were reduced to flakes having an average length of 20 mm and an average width of 15 mm. The flakes were conveyed with a screw conveyor to a disc refiner, where the flakes were defibrated to fluff.

Samples were taken and analysed in accordance with the aforegoing. The results obtained are shown in Table 2 below.

As will be seen from the Table, less energy was consumed when applying the invention. When compared with the use of solely sulphite pulp, as in Example 1, the admixture of groundwood pulp with sulphite pulp resulted in a surprisingly low energy consumption. As will also be seen from the Table, the qualities of the product produced by the method according to the invention were better throughout. The lower spread in diaper weight obtained was also particularly surprising.

The invention is not restricted to the afore-described embodiments. Thus, subsequent to drying and shredding the pulp it can be mixed with another dried and shredded pulp of different quality, i.e. sulphate pulp or a thermo-mechanical pulp. It is also possible within the scope of the invention to mix the dried and shredded pulp with conventional flash dried pulp. Examples of other types of fibre which can be mixed with the dried and subsequently coarsely shredded pulp include recycled fibres and synthetic fibres.

Large units other than straight-sided bales can also be used in accordance with the invention. Thus, it is also possible to manufacture large units by filling the dried and coarsely-shredded pulp into plastic packages of different shapes and sizes and compress the packages to the density desired.

### Example 3

In a sulphite mill, in which there was produced 2-stage-cooked, fully bleached spruce sulphite pulp having an intrinsic viscosity of 1100 cm³/g and a brightness of 93% ISO, a defibrating means was installed downstream of a drying machine, for disintegrating the pulp web. The defibrating means comprised a rotatable roller provided with sharp pyramidal spikes. The defibrating means is usually called a spiked roller and is normally used for coarsely shredding moist pulp prior to flash drying the same in a conventional manner.

The dry solids content of the pulp during the disintegrating operation was 93.5%, and flakes were obtained having an average width of about 15 mm and an average length of about 20 mm. The pulp flakes were charged to a slab press and then to a bale press. During the test, large units in the form of straight-sided bales having a weight of 180 kg bone dry pulp were produced. The bales were 47 cm in height, 91 cm in length and 65 cm in width. This gave each bale a density of 650 kg/m³. After being conditioned for two weeks, the flake bales were transported to a converting plant for the manufacture of diapers. The bales then had a dry solids content of 91.5%. The bales containing said flakes were opened in the plant and torn into small pieces by means of a simple peg shredder. The pieces obtained were identical in size and number to the flakes obtained prior to baling in the pulp mill. The pulp flakes were conveyed in a screw conveyor to a disc refiner, in which they were defibrated to fluff form. It could be noted during the test that the pulp bales were readily torn apart and that the pulp flakes were readily defibrated. It was also noted that difficulties due to static electricity were considerably less than normal. Diapers weighing about 32 g were manufactured during the test. The spread in diaper weight was ±1 g, and was fully satisfactory. The bulk and absorption properties of the pulp were checked prior to producing the diapers. The result is given in Table 3 below.

To enable comparisons to be made, pulp sheets were taken from the mill and stacked and compressed in a conventional manner into bales having the aforementioned measurements. The bales weighed 190 kg (bone dry) and their density was 685 kg/m^{3.} The dry solids content of the pulp immediately after the web dryer was 93%. After being conditioned for two weeks, the dry solids content was 92.0%. The pulp bales were then transported to the converting plant where they were cut into strips on the guillotine. The strips had a width of 5 cm and a length of 80 cm. The pulp strips were fed on a belt conveyor to a hammer mill, where they were reduced to flakes having an average length of about 20 mm and an average width of about 15 mm. The pulp flakes were conveyed in a screw conveyor to a disc refiner, where the flakes were defibrated to fluff. No difficulties were experienced in manufacturing diapers from the defibrated pulp, with the exception of certain problems with static electricity. Diapers manufactured during the test weighed about 32 g. The diaper weight spread was 11g.

The bulk and absorption properties of the pulp were checked immediately after defibration, i.e. just prior to manufacturing the diapers. The results are given in the Table below. All measurements have been made in accordance with Scan-C 33:80.

As will be seen from the Table, the energy consumed is lower then that consumed when shredding and defibrating pulp according to conventional methods, even when the pulp web is shredded by means of a spiked roller. In addition, there is obtained a better end product.

## Claims

1. A method for manufacturing a cellulose pulp material suitable for further processing to absorbent products in a converting plant, whereby dried cellulose pulp web is used as basic material, characterized by disintegrating the dried cellulose pulp web into flakes directly in the pulp mill; and by compressing the resultant flakes into large easily handled and transportable units having an apparent density of 200-800 kg/m³, preferably 300-700 kg/m³.

2. A method according to Claim 1, characterized by disintegrating at least 70% of the dried pulp web into pieces (flakes) having an average width/length or average diameter of 2-70 mm, preferably 3-40 mm.

3. A method according to Claims 1-2, characterized in that the dried pulp web has a dry solids content of at least 80% when leaving the drying machine.

4. A method according to Claims 1-3, characterized by cutting the dried pulp web leaving the drying machine into sheets; stacking the sheets loosely one upon the other; cutting the stack of sheets into strips; disintegrating said strips into flakes, and compressing said flakes to form large units.

5. A method according to Claims 1-3, characterized by disintegrating the dried pulp web into flakes immediately upon leaving the drying machine, and compressing said flakes to form large units.

6. A method according to Claims 1-5, characterized by conditioning the large flake units formed in the pulp mill before their transport to a converting plant for shredding into fluff and manufacture of absorbent products.

7. The use of the cellulose pulp material obtained in the method of any of claims 1-6 for the production of absorbent products in converting plants.

## Patentansprüche

1. Verfahren zur Herstellung eines Zellulose-Halbstoffmaterials, das zur weiteren Verarbeitung zu absorbierenden Produkten in einer Umwandlungsanlage geeignet ist, wobei eine getrocknete Zellulose-Halbstoffbahn als Grundmaterial verwendet wird, gekennzeichnet durch Auftrennten der getrockneten Zellulose-Halbstoffbahn in Flocken direkt in der Halbstoffmühle und durch Verdichten der erhaltenen Flocken zu großen, leicht handhabbaren und transportablen Einheiten mit einer Rohdichte von 200 bis 800 kg/m³, vorzugsweise 300 bis 700 kg/m³.

2. Verfahren nach Anspruch 1, gekennzeichnet durch Auftrennen von mindestens 70% der getrockneten Halbstoffbahn in Stücke (Flocken) mit einer mittleren Breite/Länge oder einem mittleren Durchmesser von 2 bis 70 mm, vorzugsweise 3 bis 40 mm.

3. Verfahren nach den Ansprüche 1 bis 2, dadurch gekennzeichnet, daß die getrocknete Halbstoffbahn einen Trockkenfeststoffgehalt von mindestens 80% beim Verlassen der Trocknungsmaschine hat.

4. Verfahren nach den Ansprüchen 1 bis 3, gekennzeichnet durch Schneiden der getrockneten Halbstoffbahn beim Verlassen der Trocknungsmaschine zu Bögen; lockeres Aufeinanderstapeln der Bögen; Schneiden des Stapels von Bögen zu Streifen; Auftrennen der Streifen in Flocken und Verdichten der Flocken, um große Einheiten zu bilden.

5. Verfahren nach den Ansprüchen 1 bis 3, gekennzeichnet durch Auftrennen der getrockneten Halbstoffbahn in Flokken unmittelbar beim Verlassen der Trocknungsmaschine und Verdichten der Flocken, um große Einheiten zu bilden.

6. Verfahren nach den Ansprüchen 1 bis 5, gekennzeichnet durch Konditionieren der in der Halbstoffmühle gebildeten großen Flockeneinheiten vor deren Transport zu einer Umwandlungsanlage für das Verfasern zu Fluff und die Herstellung von absorbierenden Produkten.

7. Verwendung des Zellulose-Halbstoffmaterials, erhalten in dem Verfahren nach irgendeinem der Ansprüche 1 bis 6, zur Herstellung von absorbierenden Produkten in Umwandlungsanlagen.

## Revendications

1. Procédé de fabrication d'une matière de pâte cellulosique convenant à la transformation ultérieure en produits absorbants dans une installation de conversion, dans lequel on utilise comme matière fondamentale une bande de pâte cellulosique séchée, caractérisé par le fait que l'on désagrège en flocons la bande de pâte cellulosique séchée directement dans l'usine de pâte et que l'on comprime les flocons obtenus en grandes unités faciles à manier et transportables, ayant une masse volumique apparente de 200 à 800 kg/m³, de préférence de 300 à 700 kg/m³.

2. Procédé selon la revendication 1, caractérisé par le fait que l'on désagrège au moins 70% de la bande de pâte séchée en morceaux (flocons) ayant une largeur/longueur moyenne ou un diamêtre moyen de 2 à 70 mm, de préférence de 3 à 40 mm.

3. Procédé selon l'une ou l'autre des revendications 1 ou 2, caractérisé par le fait que la bande de pâte séchée a une teneur en solides secs d'au moins 80% lorsqu'elle quitte le séchoir.

4. Procédé selon l'une quelconque des revendications 1 à 3, caractérisé par le fait que l'on coupe en feuilles la bande de pâte séchée quittant le séchoir, que l'on empile librement les feuilles l'une sur l'autre, que l'on coupe la pile de feuilles en bandelettes, que l'on désagrège les bandelettes en flocons et que l'on comprime les flocons pour former de grandes unités.

5. Procédé selon l'une quelconque des revendications 1 à 3, caractérisé par le fait que l'on désagrège en flocons la bande de pâte séchée immédiatement à la sortie du séchoir et que l'on comprime les flocons pour former de grandes unités.

6. Procédé selon l'une quelconque des revendications 1 à 5, caractérisé par le fait que l'on conditionne les grandes unités de flocons formées dans l'usine de pâte avant de les transporter à une installation de conversion pour le déchiquetage en bourre et la fabrication de produits absorbants.

7. Utilisation de la matière de pâte cellulosique obtenue selon le procédé revendiqué dans l'une quelconque des revendications 1 à 6, pour la fabrication de produits absorbants dans des installations de conversion.
